

Feb. 7, 1939.

F. R. SEAWEY ET AL

2,146,033

HANDLING OF SENSITIVE MATERIALS

Filed Feb. 28, 1935



Fig. 1.



Fig. 2.



Fig. 3.

Inventors

FREDERICK R. SEAWEY & EDWARD B. W. KERONE

By John H. Brumley  
Attorney

## UNITED STATES PATENT OFFICE

2,146,033

## HANDLING OF SENSITIVE MATERIALS

Frederick R. Seavey and Edward B. W. Kerone,  
Alton, Ill., assignors to Western Cartridge Cor-  
poration, East Alton, Ill., a corporation of Del-  
aware

Application February 28, 1935, Serial No. 8,598

## 4 Claims. (Cl. 52—19)

This invention relates generally to the han-  
dling of sensitive or hazardous materials, such as  
explosives and particularly to a process of dehy-  
drating such materials without permitting them  
5 to become free of desensitizing or deterrent  
liquid.

Most explosives are purified, manufactured, or  
precipitated in aqueous solution and it is highly  
desirable particularly with reference to highly  
10 sensitive explosives and other hazardous mate-  
rials, such as mercury fulminate, lead azide, lead  
styphnate, powdered zirconium and the like, that  
these materials be maintained in a wet condi-  
tion during the manufacturing and mixing proc-  
15 esses and in fact until they are deposited in the  
final housing or component. As pointed out in  
the prior copending application, Serial No.  
595,418, filed February 26, 1932, now Patent No.  
2,000,995, patented May 14, 1935, of which this  
20 application is a continuation in part, the use of  
water as the wetting medium has the disadvan-  
tage that the water evaporates rather rapidly so  
as to leave particles of the explosive in a dry and  
hazardous condition. In the application men-  
25 tioned, a process is disclosed whereby the water  
with which sensitive materials are wet may be  
removed by first washing the water-wet material  
with a liquid, such as alcohol which is miscible  
30 with water until the water is removed from the  
sensitive materials and thereafter replacing the  
alcohol with a relatively non-volatile medium  
such as dichlor-ethyl ether.

It is among the objects of the present inven-  
tion to provide a process of handling water-wet  
35 materials whereby the materials may be trans-  
ferred directly from water to a medium of rela-  
tively low volatility without an intermediate dry-  
ing stage.

A further object of this invention is to provide  
40 a process of rendering hydrophilic materials or-  
ganophilic.

Another object of this invention is to provide  
a process and apparatus for dehydrating organo-  
philic materials without permitting them to dry.

45 Another object of this invention is to provide  
a process of handling sensitive or hazardous ma-  
terials whereby the materials may be transferred  
directly from water to a liquid vehicle of com-  
50 paratively low volatility without an intermediate  
relatively hazardous stage.

A more specific object of this invention is to  
provide a process and apparatus in which a hy-  
drophilic explosive may have its surface modi-  
55 fied so as to become organophilic and thereby

facilitate replacing the water directly with an  
organic medium.

Other objects will become apparent to those  
skilled in the art when the following description  
is read in connection with the accompanying 5  
drawing illustrating elemental apparatus suit-  
able for carrying out the processes of the present  
invention.

Figure 1 is a diagrammatic view showing one  
form of apparatus for carrying out the processes 10  
of the present invention.

Figure 2 is a diagrammatic view showing a  
modified form of apparatus for carrying out the  
processes of the present invention.

Figure 3 is a view more or less diagrammatic 15  
in form showing a centrifuge particularly  
adapted for carrying out the processes of the  
present invention.

In accordance with the present invention, gen-  
erally stated, a sensitive material which is nor-  
mally water-wet and which in addition has a  
surface hydrophilic in character, that is to say,  
is preferentially wet by water rather than by  
certain organic liquids, may be treated with an  
agent capable of so modifying the surfaces of 20  
the particles that their surfaces become organo-  
philic. With the surface thus modified the water  
with which the material has been wet may be  
readily removed by incorporating the mixture  
with the organic liquid which it is desired to em-  
ploy. After thorough incorporation, if the mix-  
ture be permitted to stand, the particles of sensi-  
tive material will become entrained in the or-  
ganic liquid while the water segregates so that it  
may be separated by decantation, centrifuging, or  
otherwise. Moreover centrifugal separation may  
be accomplished immediately after incorporation. 30

Such explosive and sensitive substances as lead  
azide, powdered zirconium, etc., are normally  
40 hydrophilic. In accordance with the present in-  
vention, however, these materials when treated  
with long chain fatty or long chain unsaturated  
acids, such as palmitic, stearic, oleic, linolenic,  
or linoleic acids, etc., or by soluble soaps, appear  
45 to have their surfaces modified so that they be-  
come organophilic and hence the water in which  
they are incorporated may be directly replaced  
by an organic liquid having the desired proper-  
ties such as a lower volatility than water and a  
greater protective action generally. Examples 50  
of such organic liquids which may be advantage-  
ously used in connection with such explosive and  
sensitive materials are dichlorethyl ether, tetrachlo-  
rethylene, trichlorethane, and tetrachlor-  
55 ethane.

Such organophilic-coat-producing agents as the long chain fatty and long chain unsaturated acids and their alkali soaps may be applied to the explosive materials in various ways. For instance, the long chain fatty and long chain unsaturated acids may be emulsified in water and this emulsion incorporated in a water slurry of the explosives. In the case of the soluble alkali soaps of these acids, however, a solution thereof 5 may be made with water and this solution incorporated with a water slurry of the explosive. As another alternative, either the acid or the soap may be incorporated in the organic liquid which is subsequently to be mixed with the water slurry 10 of the explosive. In each instance, however, care should be taken to sufficiently incorporate or mix the media containing the organophilic-coat-producing agent so that each particle of the explosive is contacted with that agent. Emulsifying 15 agents may be used to facilitate the preparation of suitable emulsions when advantageous.

Such organophilic-coat-producing agents appear to react slightly with the material so as to produce a heavy metal soap of the acid employed 20 upon the surface of the particles of the material. An extremely small proportion of organophilic-coat-producing agent is necessary in order to produce a coating which, for the purpose, obviously may be extremely thin. Since such heavy 25 metal soaps are readily wet by organic liquids but are not wet by water, it will be understood that the particles of explosives are rendered organophilic so that when an organic liquid is incorporated with the water slurry of the explosive 30 the particles, being preferentially wet by the organic liquid, desert the water or become enveloped by the organic liquid so that a suspension of the explosive in the organic liquid results.

As a specific illustration take, for instance, 35 water-wet lead azide as the material to be treated, dichlorethyl ether as the organic liquid, and oleic acid as the organophilic-coat-producing agent. One part of lead azide suspended in ten parts of water may be treated with a water emulsion of oleic acid containing 0.75% oleic acid (based on the dry weight of lead azide) and one part of water. The emulsion may be added to the lead azide-water slurry and vigorously agitated in order to assure an even distribution of oleic 40 acid over the lead azide particles. To this mixture may then be added ten parts of dichlorethyl ether (the organic liquid) and the entire mixture may be stirred sufficiently to assure that every particle of lead azide has been contacted with 45 the dichlorethyl ether. The mixture may now be separated by any suitable method such, for instance, as by centrifuging or by settling and decantation. If for instance, the mixture is centrifuged so as to remove the excess liquid the lead 50 azide will remain behind in the form of a paste completely dehydrated but wet with the dichlorethyl ether.

As another embodiment instead of employing the emulsion of oleic acid as described above, a 55 solution of sodium oleate, triethanolamine oleate or other water soluble soap containing about 0.75% of oleate or other long chain unsaturated or fatty acid in water may be substituted. In this case, as in the example above, upon the addition of the organophilic-coat-producing agent 60 the lead azide slurry is thoroughly agitated so as to assure even distribution thereof. Thereafter the organic liquid, such as dichlorethyl ether, may be added and the excess liquid removed as in the previous illustration.

As another specific example the organophilic-coat-producing agent may be directly dissolved in the dichlorethyl ether. For instance, a solution may be made in ten parts of dichlorethyl ether containing 0.75% of oleic acid (based upon 5 the dry weight of the lead azide) and this solution incorporated directly with the lead azide water slurry. The agitation and separation steps described above are again carried out.

Normally organophilic explosives which have 10 become wet with water may be dehydrated by drowning in a bath of organic liquid or otherwise incorporating sufficient organic liquid to displace the water.

As illustrating the dehydration of mercury 15 fulminate, for example, a slurry composed of 100 parts of fulminate in 500 parts of water may be treated with a solution of 1 to 2 parts of potassium ethyl xanthate in 10 parts of water. The xanthate solution is thoroughly mixed with the 20 slurry and thereafter about 500 parts of dichlorethyl ether may be mixed in. The fulminate then settles with the dichlorethyl ether and the water may be decanted off. Of course, other 25 organophilic-coat-producers, as described above, may be used instead of potassium ethyl xanthate.

Referring now particularly to the drawing for an illustration of various forms of apparatus suitable for carrying out the processes of the present invention the apparatus shown in Figure 1 may 30 comprise a receiving jar 1 and a mixing vessel 2. As shown, the mixing vessel is formed as an inverted cone having a neck 3 which extends into the receiving jar. A suitable stopper 4 may be provided for sealing the space between neck 3 and 35 the neck of jar 1. Another stopper 5 is provided for closing the neck of mixing vessel 2 on the inside and this stopper may be conveniently provided with a long rod 6 by which it may be readily seated and unseated. A suitable agitator 7 is also 40 provided.

In carrying out the invention in accordance with this embodiment jar 1 may be filled with the organic liquid such as dichlorethyl ether to a level such that the end of neck 3 will be submerged and 45 stopper 4 may then be inserted so as to leave a small air space between the level of the liquid and the stopper 4. Additional dichlorethyl ether is now poured into dehydration vessel 2 so as to fill neck 3 and the stopper 5 is then inserted. After stopper 5 is inserted the desired amount of dichlorethyl ether, such for instance as sufficient 50 to extend up to level 8, may be added. The water slurry containing the explosive such as lead azide may now be placed in vessel 2 so as to bring the 55 level thereof up to 9. Agitation is now begun, it being understood that the organophilic-coat-producing agent is included in either the organic medium placed in vessel 2 or in the slurry as hereinbefore described. The agitation may be 60 continued until all of the lead azide has settled into the organic liquid. In case the water and organic liquid tend to emulsify, slow agitation in the interface will be found to break the emulsion and if globules of water become occluded 65 in the organic liquid, they may be freed by upward agitation in the organic liquid face. When the lead azide has all settled from the water phase to the organic phase, stopper 5 may be removed so as to permit the azide to settle further 70 down into the receiving vessel 1 leaving the water above level 8.

A modified form of apparatus in which separation of entrained occluded water is more certain is illustrated generally in Figure 2. In ac-

cordance with this embodiment a receiving jar 11 is provided as before. Into the mouth of receiving jar 11 is fitted an immersion vessel 10 provided with a neck 13 and a stopper 15 having a control rod 150 for the interior thereof. Within the immersion vessel 10 is contained a smaller mixing vessel 12 which, as in the previous embodiment, is provided with an agitating device 17 and a stopper 16 for mouth 120.

10 In the use of this form of apparatus the receiving jar and the immersion vessel are filled with dichlorethyl ether and, as in the previous embodiment, stopper 15 is seated. The stopper 16 in mixing vessel 12 is also seated and additional dichlorethyl ether is poured therein so as to bring the level thereof up to 18. Upon the dichlorethyl ether in the mixing vessel may be poured the water slurry so as to bring the water up to the level 19. In the use of this apparatus the incorporation and agitation is accomplished as before, but when the lead azide has settled into the organic medium, stopper 16 is removed so as to permit the same to pass into the dichlorethyl ether contained in immersion vessel 10 and here again the mixture stands until the lead azide settles to the bottom. During this settling period it will be understood that opportunity is afforded for globules of entrained or occluded water to segregate and rise to the top in immersion vessel 10. It may also be pointed out that the various vessels may be made of glass or so arranged that the levels of the liquids may be ascertained.

When the azide has finally settled in immersion vessel 10 stopper 15 may be lifted to permit the same to be further settled into the receiving jar 11. After such settling stoppers 15 and 16 may be replaced and jar 11 removed.

Another form of apparatus which may be used is shown in Figure 3. In this case one or more cups 20 may be suitably mounted as by a support 21 to a shaft 22 which may be rotated. Cups 20 may be pivotally connected to support 21 as shown at 23 so as to permit them to swing into the dotted line position upon rotation of the shaft. It is also convenient to mount the cups so that they may be readily removed. Cups 20 may be provided with a suitable lining such as rubber.

In the use of this form of apparatus, for example, the water wet slurry of explosive is placed into cups 20. The required amount of oleic acid is then added as a water emulsion with stirring, followed by the addition of the required amount of dichlorethyl ether also with stirring. The rubber cups are then placed in the centrifuge and centrifuged slowly to break the emulsion and release the occluded water, after which the centrifuge is turned to higher speed for the required length of time to pack the explosive to a paste of the required solids content. If found desirable in order to remove final traces of water which may be occluded, the explosive may be resuspended in fresh dichlorethyl ether and recentrifuged. The paste thus obtained is then ready for storage or use.

From the foregoing description it is apparent that processes hereinbefore described accomplish the objects of the invention and that water wet explosive may be dehydrated in accordance with the present invention by direct replacement of the water with a suitable organic medium. As pointed out hereinbefore for the handling of explosives, dichlorethyl ether, tetrachlorethylene, trichlorethane and tetrachlorethane are ideal because they are relatively difficult to ignite and of considerably lower volatility than water and

hence will not tend to evaporate and leave dry particles of explosive during the manufacturing and handling stages.

Although for the purpose of illustration the foregoing description has been confined to the use of the processes with lead azide it is to be understood that the processes are applicable alike to other highly sensitive explosives and hazardous materials, such for instance as mercury fulminate, lead styphnate, basic lead azide, nitrosoguanidine, tetracene, guanyl tetrazyl triazene, potassium azinol, basic lead styphnate, lead and silver azinol, powdered zirconium, etc. In these cases except the latter, water is present from the manufacturing operations since with 15 these materials some stage of manufacturing, purification or precipitation is conveniently carried out with the substances in aqueous solution. In the case of zirconium powder, however, this material may be produced by wet grinding and it 20 will be understood that the water from the grinding operation may be supplanted with a suitable organic medium, such as dichlorethyl ether, either directly in accordance with the present invention, or indirectly by the use of an intermediate washing with alcohol as described in the 25 copending application Serial No. 595,418.

For instance direct dehydration of zirconium powder may be facilitated by a preliminary activating treatment using a substance which will 30 bind the organo-philic-coat-producing agent to the surface of the particle. Silver nitrate may be employed as the activator in this case and thereafter either oleic acid which for convenience may be in an alcohol solution or potassium ethyl 35 xanthate in aqueous solution or other suitable agent may be applied as above described to produce the organophilic coat which enables the organic liquid to envelope the particles. Direct dehydration of nitrosoguanidine, tetracene and 40 guanyl tetrazyl triazene is readily accomplished by using activators. Lead nitrate and nickel nitrate are particularly useful when the aqueous suspension of these materials is made slightly 45 ammoniacal.

Such activators may be used with advantage wherever an organophilic-coat-producer which will react with the solid is not at hand. Even with some materials which can be dehydrated without activators, the operation is expedited by 50 the use of activators. In such cases the activator may react with the solid to produce a film with which the other agent may react to produce the surface condition.

The organic liquid employed for desensitizing 55 should be selected so as to avoid solution of the coats on the solid or the solid itself. For instance, in dehydrating potassium azinol using lead nitrate as the activator, a coat of lead azinol is produced. Since this coat is somewhat soluble in dichlorethyl ether another liquid, such for instance as ethyl acetate may be used and after the solid has been wet the dichlorethyl ether may be added. Likewise, dehydration of nitrosoguanidine and tetracene proceed smoothly when ethyl acetate is used followed by dichlorethyl ether.

By the expression "organophilic coating substance", as used herein and in the appended claims, as well as similar expressions which may 70 be found therein, it is intended to include those substances which either by surface reaction or adsorption convert the surface of the particles of explosives from a character in which they are preferentially wet by water to a character in

which they are preferentially wet by an organic liquid to be employed.

Since it is apparent that the process and apparatus hereinbefore described are applicable to various fields of use and are susceptible to many modifications of the specific procedure hereinbefore described which will immediately present themselves to those skilled in the art, it is to be distinctly understood that the invention is not limited to the details of the processes and apparatus herein disclosed, but that such modifications and the use of such individual features and subcombinations of features as do not depart from the spirit of this invention are, although not specifically described herein, contemplated by and within the scope of the appended claims.

Having thus described the invention what is claimed is:

1. In the art of handling explosives having a high order of sensitivity such as lead azide and which are unsafe for handling in the form of water-wet paste, the process comprising, providing a water slurry of the explosive, adding to the slurry an organophilic coat producing substance, incorporating an organic liquid which is inert to the explosive, less volatile than and immiscible with water, and removing the water.

2. The art of handling explosives having a high order of sensitivity such as lead azide and which are unsafe for handling in the form of water-wet paste, the process comprising, providing a water slurry of the explosive, adding to

the slurry an organophilic coat producing substance of the class consisting of alkali xanthates, long chain fatty acids, long chain unsaturated fatty acids and water soluble soaps thereof, incorporating an organic liquid which is inert to the explosive, less volatile than and immiscible with water, and removing the water.

3. In the art of handling explosives having a high order of sensitivity such as lead azide and which are unsafe for handling in the form of water-wet paste, the process comprising, providing a water slurry of the explosive, treating the explosive with a metal activator, treating the activated particles of explosive with an agent whose reaction product with the activated surface of the explosive is organophilic, incorporating an organic liquid which is inert to the explosive, less volatile than and immiscible with water, and removing the water.

4. In the art of handling explosives having a high order of sensitivity such as lead azide and which are unsafe for handling in the form of water-wet paste, the process comprising, providing a water slurry of the explosive, adding to the slurry an organophilic coat producing substance, incorporating an organic liquid which is inert to the explosive, less volatile than and immiscible with water, centrifuging the resultant product to obtain a paste wet with the organic liquid, and removing the water.

FREDERICK R. SEAVEY.  
EDWARD B. W. KERONE.